

Jan. 18, 1927.

1,614,670

W. E. GREENAWALT

COPPER EXTRACTION PROCESS

Filed June 8, 1926



INVENTOR  
William E. Greenawalt

Patented Jan. 18, 1927.

1,614,670

# UNITED STATES PATENT OFFICE.

WILLIAM E. GREENAWALT, OF DENVER, COLORADO.

## COPPER-EXTRACTION PROCESS.

Application filed June 8, 1926. Serial No. 114,477.

The process has as its object the production of electrolytic copper from its ores without resorting to regular smelting and refining methods, which, in most mining 5 districts, are too expensive for general adoption.

The following considerations are the principal factors governing the process, and when these are understood the process can 10 be easily comprehended.

In leaching copper ore with an acid solution, such as sulphuric acid, iron is always dissolved with the copper. In the electrolysis of copper solutions containing salts 15 of iron, copper is deposited while sulphuric acid and ferric iron are regenerated, as shown by the following equation:



in which  $x$  represents an indeterminate amount of sulphuric acid and  $y$  an indeterminate amount of ferric sulphate. The relative amounts of acid and ferric sulphate 25 produced by the electrolysis will largely depend on the details of operation, such as the iron content of the electrolyte, the temperature of the electrolyte, and the composition of the anodes. Lead anodes, for example, 30 will usually give a relatively large amount of sulphuric acid with a relatively small amount of ferric sulphate, while carbon anodes will usually give a relatively large amount of ferric sulphate with a relatively 35 small amount of sulphuric acid.

Ferric sulphate in the electrolyte is harmful; it re-dissolves copper somewhat in proportion to its presence in the electrolyte. Ferrous sulphate is quite harmless, and it 40 may be beneficial. The crucial problem of the deposition of copper from solutions containing salts of iron, practically resolves itself to the control, or reduction, of the ferric iron produced in the deposition of the 45 copper. There are a number of practical reducing agents available for this purpose, among which may be mentioned, sulphur dioxide, metallic copper, and copper sulphide. The present process is directed more 50 particularly to a specific and economical application of copper sulphide, as related to the general treatment of the ore.

The reduction of ferric iron becomes more difficult as the solution increases in acidity.

55 Ferric sulphate is easily reduced in neutral

or slightly acid solutions, while its effective reduction in highly acid solutions is very difficult. For this reason the solution should not contain an excessive amount of acid unless a large amount of acid is desired for 60 other purposes.

Sulphur dioxide is an effective reducing agent for ferric iron under some conditions if properly applied, as for example, as set forth in my patents No. 1,353,995, Sept. 28, 1920, and No. 1,483,056, Feb. 5, 1924. If ferric sulphate is reduced with sulphur dioxide a large amount of acid is regenerated, as shown by the equation,



Frequently such a regeneration of acid is desirable for leaching purposes, but it also frequently happens that it may be objectionable, especially in the treatment of high grade ore or concentrate where the acid consumption is relatively small. 75

If the ferric iron is reduced with copper sulphide, as set forth in some detail in my 80 patents, No. 1,340,826, May 18, 1920, No. 1,357,495, Nov. 2, 1920, and No. 1,489,121, Apr. 1, 1924, copper goes into solution with the simultaneous reduction of the ferric iron, while little or no acid is regenerated, 85 as shown by the equations:



The copper sulphide may be either the 90 natural sulphide, such as chalcocite, covellite, or chalcopyrite; a high grade copper matte as obtained from smelting; or a precipitate obtained by precipitating copper from lean and foul solutions with a sulphide precipitant such as hydrogen sulphide.

The application of sulphur dioxide to the leach solution, or electrolyte, is usually advantageous, but it will be seen that if the electrolysis is conducted in such a way as 100 to generate a maximum amount of ferric iron and a minimum amount of acid, and the ferric iron is reduced with copper sulphide, a considerable saving would result over other methods of procedure, for the 105 reason that copper would go into solution at the expense of the ferric iron and would be deposited as the electrolytic metal, while the acidity of the solution could be kept under control. A wide range of operating 110

conditions could thus be maintained by increasing or diminishing the variable factors of the process.

Carbon anodes, if they can be used, would regenerate a maximum amount of ferric iron and a minimum amount of acid. If carbon anodes are used it is desirable to have a warm or hot electrolyte and vigorous circulation or agitation to facilitate de-polarization, which appears to be essential for the preservation of carbon anodes and the generation of large quantities of ferric iron in the deposition of copper from copper solutions containing salts of iron. But whether carbon, lead, or other anodes are used, it is desirable to maintain the temperature of the solution fairly warm, because both the deposition of the copper and the reduction of the ferric iron with copper sulphide are better with hot or warm solutions than with cold solutions.

Ferric sulphate is a solvent for copper in its sulphide combinations, while sulphuric acid is not. It might be said that the hotter the solution of ferric sulphate the more effective it is as a solvent for copper in its sulphide combinations, and the more effective ferrous sulphate is as a depolarizer in the deposition of the copper. Hot solutions are not always desirable, but under the conditions of this process hot solutions can be economically maintained and present certain advantages.

As another condition entering into the process in the treatment of sulphide concentrates, for example, roasting is an important matter. Under certain conditions of roasting it has been found that from 75% to 85%, or more, of the copper can be made soluble in water by roasting, and that a very high total extraction of the copper is possible with such a roast. But, with a large percentage of water soluble copper due to roasting, the amount of acid regenerated in the deposition of the copper should be maintained low for the most satisfactory operation. The excess acid to be wasted should be maintained as low as possible, unless oxidized ore is available for its use and neutralization, and oxidized ore is not always available in the treatment of sulphide concentrates.

As a result of these considerations and conditions, it has been found that a simple and effective process can be applied to the treatment of many or most copper ores, in which the ore itself will largely or mostly supply the essentials, if these essentials are properly manipulated.

The process will now be described somewhat in detail, reference being made to the accompanying drawing which is a flow sheet in diagrammatic plan of the process.

In describing the process, the ore to be treated may be presumed to be a sulphide, or

a sulphide containing oxides which is commonly known as a mixed ore. The ore as it comes from the mine is ground to the desired fineness and concentrated. The concentration may be done either by gravity or flotation or by both gravity and flotation combined. The sulphides are separated from the gangue which may or may not contain sufficient oxide or carbonate of copper to warrant further treatment.

The copper sulphide concentrate is divided into a high grade and a low grade concentrate, and given somewhat separate, although related, treatment. In the concentration treatment of copper ore, either by gravity or flotation or both combined, a certain amount of very high grade concentrate may be separated from the large amount of ordinary sulphide concentrate or from the ore, but the relatively small amount of high grade concentrate will contain a relatively large amount of the total copper. Usually this relatively small portion of high grade concentrate will be in the form of chalcocite, with probably relatively small amounts of bornite and chalcopyrite, which will contaminate the high grade concentrate with a small amount of iron, but not enough to effect the present process.

The copper in what is known as porphyry or disseminated deposits is largely in the form of chalcocite,  $\text{Cu}_2\text{S}$ , and contains, theoretically, 79.8% copper and 20.2% sulphur.

The conditions of concentration can best be illustrated by taking a specific case in the treatment of 100 tons of ore assaying 1.5%, or 30 pounds of copper per ton, or containing a total of 3000 pounds of copper. If the ratio of concentration is 10 into 1, the result of the concentration treatment would be about as follows:

10 tons concentrate, 12.75% copper (255 lbs.) 2,550 lbs. total.

90 tons tailing, 0.25% copper (51 lbs.) 450 lbs. total. 110

The ten tons of concentrate may then be separated into:

1.5 tons high grade concentrate, 50% copper (1,000 lbs.), 1,500 lbs. total.

8.5 tons low grade concentrate, 6.2% copper (124 lbs.), 1,050 lbs. total. 115

Or, possibly, into the following:

1.0 tons high grade concentrate, 60% copper (1,200 lbs.) 1,200 lbs. total.

9.0 tons low grade concentrate, 7.5% copper (150 lbs.) 1,350 lbs. total. 120

There should be no difficulty in making a relatively small amount of high grade concentrate, if much of the copper in the ore is in the form of chalcocite. For a 50% copper concentrate there would be a margin of 29.8% of the theoretical and for a 60% copper concentrate there would be a margin of 19.0% of the theoretical. The latter is preferred and will be assumed for illustration, 125 130

although it will be understood that the process is not particularly limited to the percentage of copper in the high grade concentrate, but that the higher the grade of the 5 concentrate the better the process can be operated. A ton of 60% copper concentrate would contain, approximately, copper, 1,200 pounds; sulphur, 400 pounds; impurities, 400 pounds. The impurities may be assumed to be mostly iron with its combined sulphur, silica, alumina, and combined oxygen.

10 If there is gold or silver in the ore, the high grade concentrate will contain the precious metals in about the same proportion as it contains the copper from the original ore. That is to say, of the total precious metal content in the concentrate, 47.5% will be in the one ton of 60% copper concentrate, 20 and 52.5% will be in the 9.0 tons of low grade concentrate assaying 7.5% copper.

25 Having made the separation of the mineral from the gangue and divided the mineral into a relatively small amount of high grade concentrate and a relatively large amount of low grade concentrate, the method of procedure is as follows:

30 The low grade concentrate is roasted so as to convert a large part of the copper into the form of sulphate, which is soluble in water, and this sulphate, on electrolysis, supplies the necessary acid for the process.

35 The roasted low grade concentrate is leached with a dilute acid solution to extract the copper. The resulting copper solution, containing salts of iron, is then electrolyzed to deposit the copper, while at the same time acid and ferric iron are regenerated. Ferric iron in the electrolyte is harmful. It redissolves copper from the cathode approximately proportional to its presence in the electrolyte. When the ferric iron in the electrolyte reaches 0.5% the deposition of the copper becomes inefficient, and when 40 it reaches 0.75% to 1.0% the process practically becomes prohibitive. For good work the solution flowing into the copper depositing tanks should be as low in ferric iron as possible, and the solution issuing from the 45 copper depositing tanks should not greatly exceed 0.25% ferric iron for good work. It may advantageously be less. For the purpose of this process the ferric iron produced by the deposition of the copper from the 50 leach solution containing salts of iron, is reduced with the high grade sulphide concentrate, consisting largely of  $\text{Cu}_2\text{S}$  and  $\text{CuS}$ . The reactions involving the reduction of the ferric iron and the solution of the copper 55 have been given in equation form.

60 By treating the copper solution obtained from the roasted low grade ore or concentrate, containing ferric iron due to the electrolytic deposition of the copper, with the raw or unroasted high grade sulphide con-

centrate, there will result several distinct advantages, among which are: first, the reduction of the harmful ferric iron to the harmless or beneficial ferrous iron which makes practical high deposition efficiency; 70

second, the copper of the high grade unroasted concentrate goes into solution simultaneously with the reduction of the ferric iron and is directly converted into the electrolytic metal; third, the expense of drying 75 and roasting the high grade concentrate, with its attendant losses, is largely if not entirely avoided, and fourth, these various factors combined result in an effectively and cheaply operating process. Copper sulphide 80

in a finely divided condition is an effective reducing agent for ferric iron, and probably its most effective form as a reducing agent is in the form of a  $\text{Cu}_2\text{S}$  or  $\text{CuS}$  precipitate, as set forth in some detail in my patents 85 No. 1,365,034, Jan. 11, 1921; No. 1,357,495, Nov. 2, 1920; and No. 1,489,121, Apr. 1, 1924. A distinct advantage however is gained by separating the high grade concentrate from the low grade concentrate and treating the 90 leach solution and electrolyte obtained from leaching the roasted low grade concentrate with the unroasted high grade concentrate as set forth in this process, although substantially the same chemical reactions are 95 involved.

It is preferred to electrolyze the copper solution obtained from leaching the roasted low grade concentrate in steps, or in a series 100 of electrolytic units. If, for example, the rich copper solution from the roasted low grade concentrate contains 4.5% copper and it is desired to impoverish it down to 2.0% copper before returning the solution to the 105 roasted concentrate, it is preferred to do it in three electrolytic units, each comprising a  $\text{Cu}_2\text{S}$  or  $\text{CuS}$  reducer and an electrolyzer, or copper tank, by taking out 1.0% of the copper in the first electrolytic unit and 0.75% in each of the remaining two. The copper 110 in the first electrolytic unit would be deposited out of an approximately 3.5% copper solution; the copper in the second electrolytic unit would be deposited out of an approximately 2.75% copper solution, and the copper in the third electrolytic unit would be deposited out of an approximately 2.0% copper solution, ignoring the copper taken 115 into solution by the ferric iron from the raw concentrate. The copper so taken into the 120 solution will vary according to the details of operation. Manifestly, such an arrangement is much better than if the electrolysis were all done in one step, which implies that the deposition would have to take place from 125 an approximately 2.0% copper solution, which, for many reasons would be highly undesirable. If the head solution is relatively low in copper, two electrolytic units, 130 composing the series, will be sufficient. If

the head solution is very high in copper, three or more electrolytic units, composing the series, may be desirable.

If the copper deposited produced the theoretical equivalent of ferric iron, then the ferric iron so produced would re-dissolve the same equivalent of copper from the raw high grade concentrate, but the theoretical equivalent is never realized, and hence the copper deposited is obtained both from the roasted low grade concentrate and from the unroasted high grade concentrate. The relative amounts will largely be dependent on the details of operation.

Some of the oxygen released at the anode will be converted into acid, and when the solution becomes excessively charged with acid, the excess acid will have to be neutralized, or a portion of the solution wasted and an equivalent of water added, or the excess acid may be used in leaching oxidized ore, which in most instances will be the tailings from the preliminary concentration process for obtaining the high grade and the low grade concentrate.

Both the acid and the iron in the solution can be largely controlled by the method of roasting the low grade concentrate. If acid is desired the roasting would be conducted to convert as much as possible of the copper into the sulphate, which, on electrolysis, will render an equivalent of acid and ferric iron. If it is desired to suppress the acid, the roasting can be conducted so that most of the copper in the roasted low grade concentrate will be in the form of oxide, which will require acid to bring the copper into solution. If iron is desired in the solution or electrolyte, the roasting would be conducted under highly sulphatizing conditions, which would give a high iron as well as a high copper solubility in water or dilute acid. If it is desired to suppress the soluble iron the roasting should be highly oxidizing. In this way the process can be largely regulated to conform with the relative amounts of high grade and low grade copper concentrate resulting from the preliminary treatment of the ore. The process works best if the high grade concentrate is largely confined to chalcocite,  $Cu_2S$ , and covellite,  $CuS$ . Chalcopyrite and bornite, or copper bearing pyrites are not as effective in reducing ferric iron as the chalcocite or covellite. While there will inevitably be some mixing of these copper minerals in the gravity or flotation concentration, the object would naturally be to have the high grade concentrate composed mostly of chalcocite and covellite with a small amount of practically pure chalcopyrite and bornite. The low grade concentrate would be composed of what is left.

It is preferred to apply the high grade copper sulphide concentrate to the electro-

lyte in a finely divided condition, in a series of  $CuS$  reducers forming part of the electrolytic units. Each  $CuS$  reducer may conveniently consist of an agitator, a separator or settling tank, and a pump to return settled fines from the settler to the agitator. Fresh concentrate may be used in all of the  $CuS$  reducers, but it is preferred to put all or most of the fresh high grade raw concentrate in the first  $CuS$  reducer, or  $CuS$  reducer No. 1, and then as the sulphide concentrate becomes impoverished in copper, pass it progressively from the  $CuS$  reducer of the first electrolytic unit to the last, and finally, when the high grade concentrate has been sufficiently impoverished in copper, the residue is added to the low grade concentrate and roasted with it to extract the remaining copper by leaching. The application of concentrated copper sulphide, obtained either as a precipitate, as chalcocite from ore, or as obtained by fusion, as a reducing agent for ferric iron produced by the electrolysis of copper solutions and the subsequent roasting and leaching of the copper sulphide residue, is set forth in some detail in my patents No. 1,340,826, May 18, 1920; No. 1,357,495, Nov. 2, 1920; No. 1,489,121, April 1, 1924; No. 1,528,207, March 3, 1925, and in my pending application, Serial No. 60,577, October 5, 1925. The present process, in this respect, is a modification or improvement to accomplish the specific purposes set forth, and may be considered as a division of my pending application Serial No. 101,194, April 10, 1926.

Various methods may be used in applying the high grade copper concentrate to the electrolyzed solution to reduce the ferric iron, but the preferred method is to finely grind the high grade concentrate and then apply it to the solution in an agitator, either of the rotary or Pachuca type, and letting the partly quiescent overflow from the agitator flow into the separator or settler to clarify the solution. The clarified solution from the settler flows into the copper tanks or electrolyzers, and the settled slime underflow is returned to the agitator. A portion of the electrolyzed solution from one electrolytic unit is returned to the agitator of the same unit, while another portion—the advance flow—is advanced to the agitator of the next electrolytic unit. In this way the solution and the high grade concentrate are advanced through the series of electrolytic units. The solution issuing from the last electrolyzer or copper depositing tank is returned to the roasted concentrate, and the residue from the high grade concentrate is added to the low grade concentrate to be roasted with it.

The reducing action of the high grade concentrate is somewhat dependent, or influenced by the temperature of the solution.

The hot roasted ore, as also the electrolysis, will tend to maintain the solution fairly warm, but in addition to this it may be desirable to maintain the temperature of the 5 solution above that due to the chemical reactions and the hot ore by applying extraneous heat.

In operating the process, the ore as it comes from the mine is separated into a 10 relatively large amount of low grade concentrate and a relatively small amount of high grade sulphide concentrate. If the concentration tailing is too lean to warrant further treatment it is wasted. If it still 15 contains values worth recovering it is transferred to the concentrate tailing leaching tank for the recovery of the remaining copper.

The low grade concentrate is roasted and 20 then leached with a dilute acid solution, preferably with sulphuric acid, to extract the copper. Iron goes into solution with the copper, and the amount of iron dissolved will depend mostly on the details of 25 roasting.

The copper solution, containing salts of iron, flows into the agitator No. 1 or settler No. 1, and from there the clear overflow passes to the electrolyzers, or copper tanks 30 No. 1, where the copper is deposited and acid and ferric iron are regenerated. The flow of the solution through the copper tanks is preferably at such a rate that the ferric iron in the effluent solution will not 35 greatly exceed 0.25%. The solution is then returned to the agitator and the cycle repeated. When the solution is agitated with the finely ground high grade copper sulphide concentrate a certain amount of the 40 concentrate slime will pass with the solution to the settler. A portion of this finely divided slime or high grade concentrate is returned to the agitator by the pump No. 1, and a certain amount, determined by 45 experience and the results desired, is advanced to the agitator of the next electrolytic unit, and so on to the third, and finally, when the high grade sulphide copper concentrate is impoverished in copper so that 50 it is no longer effective as a reducing agent, it is dewatered or filtered and added to the low grade concentrate to be roasted with it. A portion of the copper from the cells of the 55 first electrolytic unit is returned to the agitator, while another portion—the advance flow—is passed on to the second electrolytic unit, and from the second to the third or last unit, and from the third or last unit it is returned to the roasted low grade 60 concentrate where it is again reduced in acid and enriched in copper, and the cycle repeated. The amount of copper remaining in the electrolyte in passing from one electrolytic unit to the next and the number 65 of cycles in each electrolytic unit, will de-

pend on the amount of copper in the solution from the roasted low grade concentrate and the amount of copper dissolved from the raw or unroasted high grade concentrate, and the amount of acid in the solution. It 70 is not desirable to have the solution excessively high in acid.

When the solution becomes too foul for effective use, either for leaching or electrolysis, a portion is diverted from the leaching 75 and electrolytic circuit and applied to the concentrator tailing or low grade oxidized ore to extract the copper therefrom. If the resulting solution is sufficiently pure and sufficiently high in copper, it may be returned to the leaching and electrolytic circuit, with the excess acid practically neutralized. If the solution is very impure and low in copper, the solution, as also the wash water from leaching both the concentrator 80 tailing and the roasted low grade concentrate residue is treated to precipitate the copper, and the copper precipitate may be applied to the electrolyte the same as the high grade concentrate. It is preferred to 85 precipitate the copper from the lean and foul solutions with hydrogen sulphide, generated from iron sulphide and sulphuric acid, and using the resulting ferrous sulphate to regulate the iron content of the 90 leaching and electrolytic solution circuit, should more iron be desired in the solution than that furnished by the roasted low grade 95 concentrate.

I claim:

1. A copper extraction process comprising, separating copper ore into a high grade and a low grade concentrate, roasting the low grade concentrate, leaching the roasted low grade concentrate with an acid solution to extract the copper, electrolyzing the resulting copper solution containing salts of iron to deposit copper and regenerate acid and ferric iron, applying the unroasted high grade sulphide concentrate to the electrolyzed solution to reduce the ferric iron formed by the electrolysis to the ferrous condition, and then again electrolyzing the solution to deposit more copper. 100

2. A copper extraction process comprising, separating copper ore into a relatively small amount of high grade sulphide concentrate and a relatively large amount of low grade concentrate, roasting the low grade concentrate, leaching the roasted low grade concentrate with an acid solution to extract the copper, electrolyzing the resulting copper solution containing salts of iron to deposit copper and regenerate acid and ferric iron, applying the unroasted sulphide concentrate to the electrolyzed solution to reduce the ferric iron formed by the electrolysis to the ferrous condition and to dissolve copper from the unroasted high grade 110 concentrate, and then again electrolyzing the 115 solution to deposit more copper. 120

125

130

solution to deposit the copper dissolved from the roasted low grade concentrate and from the unroasted high grade concentrate as the electrolytic metal.

5 3. A copper extraction process comprising, treating copper ore to obtain a high grade and a low grade copper concentrate, roasting the low grade concentrate, leaching the roasted low grade concentrate with an acid solution to extract the copper, then alternately subjecting the resulting copper solution containing salts of iron to electrolysis and to the action of the high grade sulphide concentrate to obtain the copper of 10 both the high grade unroasted concentrate and the copper of the roasted low grade concentrate as the electrolytic metal.

4. A copper extraction process comprising, separating copper ore into a relatively 20 large amount of low grade concentrate and a relatively small amount of high grade sulphide concentrate, roasting the low grade concentrate, leaching the roasted low grade concentrate with an acid solution to extract the copper, depositing copper from the resulting copper solution containing salts of iron by alternately subjecting the solution to electrolysis and to the reducing action of the unroasted high grade concentrate, and 25 when the solution is impoverished in copper returning the solution to the roasted low grade concentrate.

5. A copper extraction process comprising, separating copper ore into a high grade 35 and a low grade concentrate, roasting the low grade concentrate, leaching the roasted low grade concentrate with an acid solution to extract the copper, electrolyzing the resulting copper solution to deposit copper and regenerate acid and ferric iron in a 40 series of electrolytic units each comprising an electrolyzer and a reducer, progressively advancing the solution from one electrolytic unit to the next of the series, and applying the high grade concentrate to the reducer of the first electrolytic unit and progressively 45 advancing it through the reducers of the series of units.

6. A copper extraction process comprising, separating copper ore into a high grade sulphide concentrate and a low grade concentrate, roasting the low grade concentrate, leaching the roasted low grade concentrate to extract the copper, electrolyzing the resulting copper solution containing salts of iron to deposit copper and regenerate acid and ferric iron, applying the unroasted sulphide concentrate to the electrolyzed solution, generating hydrogen sulphide from acid and ferrous sulphide, precipitating copper from the lean and foul solutions with the hydrogen sulphide, and adding the resulting ferrous salt to the leach solution and electrolyte.

65 7. A copper extraction process comprising,

ing, treating copper ore to separate a high grade sulphide concentrate and a low grade concentrate, roasting the low grade concentrate, leaching the roasted low grade concentrate with an acid solution to extract the 70 copper, electrolyzing the resulting copper solution containing salts of iron to deposit the copper and regenerate acid and ferric iron in a series of electrolytic units each comprising an electrolyzer and a reducer, 75 circulating a portion of the solution between the electrolyzer and the reducer of each of the electrolytic units, progressively advancing another portion of the solution from one electrolytic unit to the next, and applying the high grade sulphide concentrate to the solution in the reducers of the respective electrolytic units.

8. A copper extraction process comprising, treating copper ore to produce a high 85 grade copper sulphide concentrate and a low grade concentrate, roasting the low grade concentrate, leaching the roasted low grade concentrate with an acid solution to extract a portion of the copper, electrolyzing the resulting copper solution containing salts of iron to deposit the copper and regenerate acid and ferric iron in a 90 series of electrolytic units each comprising an electrolyzer and a reducer, circulating a portion of the solution between the electrolyzer and the reducer of each of the electrolytic units, progressively advancing another portion of the solution from one electrolytic unit to the next of the series, applying the 95 high grade copper sulphide concentrate to the solution in the reducers of the respective electrolytic units, and when the solution becomes impoverished in copper returning the solution to the roasted low grade 100 concentrate and repeating the cycle.

9. A copper extraction process comprising, treating copper ore to produce a high grade sulphide copper concentrate and a low grade concentrate, roasting the low grade concentrate, leaching the roasted low grade concentrate with an acid solution to extract the copper, electrolyzing the resulting copper solution containing salts of iron to deposit the copper and regenerate acid and ferric iron in 110 a series of electrolytic units each comprising an electrolyzer and a reducer, circulating a portion of the solution between the electrolyzer and the reducer of each of the electrolytic units, progressively advancing another portion of the solution from one electrolytic unit to the next of the series, applying the high grade copper sulphide concentrate to the solution in the reducers of the respective 115 electrolytic units, and when the high grade sulphide concentrate becomes impoverished in copper roasting the residue and leaching it to extract the remaining copper.

10. A copper extraction process comprising, treating copper ore to produce a high 120

- grade copper sulphide concentrate and a low grade concentrate, roasting the low grade concentrate, leaching the roasted low grade concentrate with an acid solution to extract 35  
5 a portion of the copper, electrolyzing the resulting copper solution containing salts of iron to deposit the copper and regenerate acid and ferric iron, applying the unroasted sulphide concentrate to the electrolyzed solution in a reducer consisting of an agitator and a settler to reduce the ferric iron formed by 40  
10 reducer, circulating a portion of the solution between the electrolyzer and the reducer of each of the electrolytic units, progressively advancing another portion of the solution from one electrolytic unit to the next of the 45  
15 series, applying the high grade copper sulphide concentrate to the solution in the reducers of the respective electrolytic units, and when the solution becomes impoverished in copper returning the solution to the 50  
20 roasted low grade concentrate to extract another portion of the copper therefrom and repeating the cycle, and when the high grade copper sulphide concentrate becomes impoverished in copper mixing the residue 55  
25 with the unroasted low grade concentrate, roasting the mixture, and leaching the roasted mixture with the impoverished electrolyzed copper solution.  
11. A copper extraction process comprising, treating copper ore to produce a high grade copper sulphide concentrate and a low 60  
30 grade concentrate, roasting the low grade concentrate with an acid solution to extract the copper, electrolyzing the resulting copper solution containing salts of iron to deposit the copper and regenerate acid and ferric iron, applying the unroasted sulphide concentrate to the electrolyzed solution in a reducer consisting of an agitator and a settler to reduce the ferric iron formed by the electrolysis to the ferrous condition, circulating the solution between the electrolyzer and the agitator and the settler and back to the electrolyzer, and returning settled solids from the settler to the agitator.

12. A copper extraction process comprising, treating copper ore to obtain a high grade sulphide copper concentrate and a low grade copper concentrate, roasting the low grade concentrate, leaching the roasted low grade concentrate with an acid solution to extract the copper, then alternately subjecting the resulting copper solution containing salts of iron to electrolysis and to the action of the high grade sulphide concentrate to obtain the copper of both the high grade unroasted concentrate and the copper of the roasted low grade concentrate as the electrolytic metal, and maintaining the solution at a temperature above that due to chemical reactions of the process.

WILLIAM E. GREENAWALT.